

Patented Apr. 19, 1927.

## UNITED STATES PATENT OFFICE.

TIETE VIERSEN, OF TER APEL, NETHERLANDS.

## METHOD OF MAKING DECORATIVE MATERIAL FROM PEAT.

No Drawing. Application filed June 1, 1926, Serial No. 113,075, and in Netherlands May 30, 1925.

Various processes are known, in which peat is pulverized or disintegrated and, if necessary deacidified and compressed in the dry or wet condition with the addition of 5 binding substances, impregnating bodies or other materials, such as gypsum, sulphur, loam, clay, calcareous sandstone, resin, alcohol, glue, tar, water glass, etc. According to all these known processes the natural 10 fibrous structure of the peat is destroyed, so that the products (for instance, plates or the like) obtained by such processes exhibit a uniform or almost uniform coloration.

The process according to the present invention is characterized by the feature, that pieces of natural bog deposit or peat ranging from 8 to 8000 cubic centimetres in size are first dried out until their water content is 10% or less and are then compressed at a 20 pressure of from 25 to 300 atmospheres.

The plates or other objects produced in this way may be polished, rubbed down, burnished or, if desired, coated with impregnating substances.

The object of the process according to the present invention is to obtain an art-decorative material of great architectural value. In consequence of the varying runs of the fibres the products obtained have a 30 wonderful color gradation or graining effect (light and shade effect), while the cost of these products is very low as a result of the cheapness of the raw materials and the inexpensive method of manufacture.

The art-decorative products obtained in this way may be used as a covering for walls,

floors and ceilings, or for the manufacture of objects of art, etc.

The process is carried out in the following 40 manner.

The pieces of bog deposit or peat are cut in sizes ranging from 8 to 8000 cubic centimetres and are then dried either by natural or artificial means until the water content is 10% or less. The dried pieces are then 45 introduced into the press without the addition of any binding or other substance so that the fibres extend in various directions and interlace with one another. The material is then pressed into the desired shape 50 at a temperature of 40-200° C. and a pressure of 25-300 atmospheres.

The pressure is dependent on the purpose for which it is desired to employ the pressed 55 material.

I claim as my invention:

A process for the production of decorative materials from pieces of peat or bog deposit having long fibres, comprising the successive steps of drying raw pieces of peat or bog in their original state to reduce their water-content to about 10%, and then pressing said pieces directly together so as to 60 consolidate them into a single integral mass or object of extreme firmness and density 65 and of the desired size in which the fibres extend in various directions throughout the mass and are caused to interlace with one another.

In testimony whereof I affix my signature.

TIETE VIERSEN.